

H. B. BRYSON,  
METALLURGICAL FURNACE,  
APPLICATION FILED SEPT. 26, 1917.

1,358,703.

Patented Nov. 16, 1920.



WITNESSES

J. H. Cabel Bradley.  
Glenn H. Leresche.

INVENTOR

Harry B. Bryson,  
By Frank H. Winter  
Attorney

# UNITED STATES PATENT OFFICE.

HARRY B. BRYSON, OF PITTSBURGH, PENNSYLVANIA.

## METALLURGICAL FURNACE.

1,358,703.

Specification of Letters Patent. Patented Nov. 16, 1920.

Application filed September 26, 1917. Serial No. 193,280.

To all whom it may concern:

Be it known that I, HARRY B. BRYSON, a resident of Pittsburgh, in the county of Allegheny and State of Pennsylvania, have 5 invented a new and useful Improvement in Metallurgical Furnaces, of which the following is a specification.

The invention relates to a process of and apparatus for reducing and refining metals, 10 more particularly for use in reducing iron ores to produce steel.

The general object of the invention is to provide an improved process of and apparatus for reducing and refining metal-bearing 15 substances.

More particularly, the object is to improve the construction and operation of furnaces by means of which, in a furnace of the open-hearth type, conditions can be created 20 which are similar to those that exist at the present time only in graphitic crucible or electric furnaces.

A further object is to provide a furnace of the open-hearth or regenerative type 25 which is so constructed that it may be easily repaired or relined, and charged and discharged expeditiously.

Other objects and advantages of the invention will appear from the following 30 specification.

A suitable apparatus by means of which the process may be carried out is illustrated in the accompanying drawing, which shows a cross section of the improved apparatus.

The process will first be described generally, and then the apparatus explained, after which the manner of carrying out the process, with the apparatus, will be set forth.

In the manufacture of steel the physical properties are governed very largely by the carbon content. It is rather difficult to accurately control the carbon content unless the iron used in making the steel is in the form 45 of pig iron of known analyses, and the entire process carried out carefully under predetermined conditions. If ore or scrap or other sources of iron are used, the carbon content is very uncertain, and the steel produced is not of uniform character. The crucible furnace and the electric furnace have been used for this purpose, but they are quite expensive and not entirely satisfactory in some respects.

The present process has been devised for producing steel of homogeneous structure.

and uniform carbon content, such as is now produced in one pot of a crucible furnace or in an electric furnace, and to effect this result by creating in a furnace, preferably 60 of the open-hearth or regenerative type, conditions similar to those existing in the crucible and electric furnace processes of making steel, thereby so altering and improving the working conditions in the open- 65 hearth furnace that it will be especially adapted to give the same or better results than are now obtained in the crucible or electric furnaces. By means of this improved process and apparatus, steel of the 70 highest grade can be produced at a much lower cost than with the use of the furnaces to which reference has been made. While the process and apparatus is particularly 75 adapted for producing steel, it may be used for refining various other metals, and, generally stated, the process and apparatus may be employed for economically reducing and refining various metals, especially reducing iron from its ore, from scrap, or from other 80 iron-bearing substances, and refining it to manufacture steel.

Conditions similar to those now existing in the crucible or electric furnace, are created in a furnace of the open hearth or similar type, by constructing the floor or bottom and portions of the sides of the furnace of graphitic bricks or blocks so arranged as to form a graphitic cup or bowl into which the metal-bearing substances are charged, 85 and having the molten metal-bearing substances in this cup or bowl covered with a vitreous slag, which acts as a lid or cover to the graphitic bowl and thus establishes improved conditions, similar to the crucible 90 and electric furnace conditions.

The furnace for carrying out this process is constructed, in a general way, similar to the present type of open-hearth furnaces, but the floor and part of the sides are made 100 of graphitic bricks which are built into the furnace in such a way as to form an integral or fixed part of the structure, the arrangement being such that the bottom of the furnace will not lift during the process of reduction and so spoil the heat or defeat the process. The graphitic floor is also made mechanically detachable so that it may be renewed or replaced and another bottom or floor substituted. The entire furnace is constructed so that the interior is readily accessible, and is also arranged so that it may be 105 110

turned or tilted into a position to allow the molten metal to be readily poured out.

The furnace comprises a lower body portion 1, and an upper or roof portion 2, the latter being erected on a steel frame 11 so that if desired it may be lifted bodily by a traveling crane or the like, to permit access to the interior for the purpose of relining the furnace or making other repairs. The lower portion is built out of brick or other suitable material, supported by I-beams 3, fixed to arcuate members 4, only one of the latter being shown in the drawing. These arcuate members rest upon rollers 5, suitably journaled on pedestals 7. An electric motor 8 is geared to an arcuate member for tilting the furnace to the necessary position for pouring the metal, through the pouring spout 9, and returning the furnace to normal position. This construction permits the entire furnace to be easily manipulated for the purpose of discharging the reduced metal.

The bottom, sides and ends of the interior of the base portion 1, of the furnace, are lined with carbon or graphitic blocks or bricks 10, as illustrated. These bricks are of good size and in addition to the carbon, contain a suitable amount of silica, or clay free from iron, or both, making them fairly hard; and preferably are positioned in the bottom of the furnace so as to form an inverted arch, thus preventing the bottom of the furnace from lifting during the heat. By building the lining in this manner, a graphitic cup or bowl is formed in which the metal may be reduced without destroying the lining during the process of reduction. The lining forms, in effect, an integral part of the furnace, but may nevertheless be removed after the furnace has been used for some time and replaced by a new lining.

This construction of furnace partly converts the open-hearth furnace into a crucible and causes the lower portion of the furnace to perform both the functions of the crucible and of the carbon electrodes of the electric furnace, namely; it acts as a container for the molten metal and maintains the molten metal in a state of fluidity, when in the final state of reduction, it is, in a carbonless state, precipitated from the bath; and is also re-carbonizes the precipitated molten metal to a desired degree; with an added advantage over the electric furnace that the heat applied to the charge is applied evenly to all parts of the charge, whereas in the electric furnace it is applied unevenly or locally by the electrodes. It is to be understood that the heat is applied in the present furnace to all parts of the furnace, as in the usual open-hearth furnace of the regenerative or open type, and preferably by the use of powdered coal as fuel.

In practising the process with this improved construction of furnace, the metal-bearing substances are placed in the graphitic cup or bowl, and, together with such limestone, silica or other flux as the nature of the charge may require, with each charge there is added a suitable amount of readily fusible earthy matter, such as kaolin, bauxite, feldspar, or any compound of aluminum, magnesium, sodium or potassium, to form a vitreous slag. Heat is then applied in the usual manner and the vitreous slag forms in the first stages of the reduction process, and, being of a lower specific gravity than the metal-bearing elements in the bath, it rises to the surface of the bath and automatically forms a lid or covering for the graphitic crucible, thereby creating crucible and electric furnace conditions.

This lid, or vitreous covering, serves two purposes: first, owing to its chemical character, it takes up and retains most of the impurities of the metal-bearing elements of the now molten mass, and, by its permeability, permits other deleterious products, such as sulfur dioxide and other gaseous products to bubble up through the covering and escape through the furnace; and, second, owing to its fluid and flexible character, it completely and automatically covers and hermetically seals and protects the molten metal of the bath against the entrance of any and all injurious, flame-borne gases of the furnace, whether oxidizing or otherwise.

It will be seen that by means of this furnace and the process employed, a furnace of the open-hearth type is constructed and utilized in such a way that it possesses all the advantages of the crucible and the electric furnaces, and may be used for producing steel directly from ores, iron scrap, or other iron-bearing substances. No pig iron need be used. When making steel of high grade or fine quality, ore or scrap of a definitely fine character will be selected.

It is to be understood that variations may be made in the exact construction of the furnace, and that the process may be used, with or without slight modifications, for reducing other metal-bearing substances. The drawings are merely illustrative and variations may be made therein and in the process, all of which are included within the invention as defined by the appended claims.

What is claimed is:

1. The process of making steel directly from iron ore, scrap, or the like, which consists in heating the iron-bearing substances in a carbon-lined furnace, and maintaining the molten metal in said receptacle covered and sealed by a vitreous slag, thereby maintaining crucible conditions in said furnace.

2. The process of making steel directly from iron ore, scrap, or the like, which con-

sists in heating the iron-bearing substances in a carbon-lined furnace, and maintaining the molten metal in said furnace covered and sealed by a vitreous slag of earthy material, thereby maintaining crucible conditions in said furnace.

3. The process of making steel directly from iron ore, scrap, or the like, which consists in heating the iron-bearing substances in a carbon-lined furnace, and maintaining the molten metal in said furnace covered and sealed by a vitreous slag of bauxite, or the like, thereby maintaining crucible conditions in said furnace.
- 10 4. The process of making steel directly from iron ore, scrap, or the like, which consists in heating the iron-bearing substances in an open hearth type of furnace provided with a carbon lining, and maintaining the molten metal in said furnace covered and sealed by a vitreous slag, thereby maintaining crucible conditions in said furnace.
- 15 5. The process of making steel directly

from iron ore, scrap, or the like, which consists in heating the iron-bearing substances in an open hearth type furnace provided with a carbon lining, and maintaining the molten metal in said furnace covered and sealed by a vitreous slag of earthy material, thereby maintaining crucible conditions in said furnace.

20 6. The process of making steel directly from iron ore, scrap, or the like, which consists in heating the iron-bearing substances in an open hearth type furnace provided with a carbon lining, and maintaining the molten metal in said furnace covered and sealed by a vitreous slag of bauxite, or the like, thereby maintaining crucible conditions in said furnace.

25 In testimony whereof I have hereunto set my hand.

HARRY B. BRYSON.

Witness:

GLENN H. LERESCHE.